

Jan. 15, 1924.

1,480,743

G. C. CARSON

METHOD OF PREVENTING SULPHUR DIOXIDE IN SMELTER GASES

Filed May 21, 1917



Fig. 2.



Fig. 1.

WITNESS:

Paul Phillips  
Carl Emerson

G. C. Carson INVENTOR.

## UNITED STATES PATENT OFFICE.

GEORGE CAMPBELL CARSON, OF SAN FRANCISCO, CALIFORNIA.

## METHOD OF PREVENTING SULPHUR DIOXIDE IN SMELTER GASES.

Application filed May 21, 1917. Serial No. 170,092.

*To all whom it may concern:*

Be it known that I, GEORGE CAMPBELL CARSON, a citizen of the United States of America, residing at 89 Broadway Street, San Francisco, California, have invented a new and useful Method of Preventing Sulphur Dioxide in Smelter Gases, of which the following is a specification.

The object of my invention is to prevent the production of sulphur-dioxide in metallurgical operations which I accomplish in the following manner. Sulphur-dioxide, when heated to temperatures ranging above the smelting temperature of the usual sulphide materials treated in metallurgical roasting and smelting operations, dissociates into sulphur and free oxygen. The temperatures which I prefer are around and above twenty-three hundred F. In practicing my invention I maintain a heated atmosphere heated to the point and above the temperature of dissociation of sulphur dioxide and pass the sulphur bearing gas through this heated atmosphere which effects the dissociation of the sulphur and the oxygen of sulphur dioxide and while dissociated I fix the oxygen of the atmosphere by spraying into it an oxidizable material to prevent it recombining with the freed sulphur vapor upon cooling.

At temperatures above the smelting point of sulphide materials  $\text{SO}_2$  breaks into  $2\text{O} + \text{S}$ ; and while dissociated I spray ore containing zinc sulphide after being ground to a fine state of division into the heated gas. The finely powdered ore gives up its sulphur to enrich the sulphur content of the gas, and the zinc becomes an oxide or soluble sulphate by combining with oxygen that would have combined with sulphur when the gas cooled sufficient to permit the combination. When zinc sulphide is not available, other sulphides can be used. The reaction that takes place is:  $\text{MS} + 4\text{O} = \text{MSO}_4$  or  $\text{MS} + 2\text{O} = \text{SO}_2 + \text{M}$ . The  $\text{SO}_2$  dissociates as soon as formed, and sets free its oxygen to combine with M thus:  $2\text{M} + 2\text{O} = 2\text{MO}$ .

Coal dust, producer gas or other carbonaceous fuels can be substituted for metallic sulphide when desired. An amount of coal dust or carbonaceous fuel should be injected into the gas before it cools to the point of formation of  $\text{SO}_2$  to insure the complete fix-

ing of the oxygen or to reduce any  $\text{SO}_2$  that forms.

Blast furnace and roaster gases are too cold to be treated by this method. Reverberatory furnace gases are generally sufficiently hot to dissociate the oxygen and sulphur of  $\text{SO}_2$ . Where side feeding and fettling furnaces are used, the furnace gas is produced at a temperature of 2400 to 2700 degrees Fahrenheit and that portion of the furnace nearest to the flue can be used for a fixing chamber to fix the oxygen and prevent its reunion with the sulphur.

The medium utilized to spray the sulphides or whatever agent is used to fix the oxygen should be a gas whose oxygen is inert, such as chimney gases or producer gas,  $\text{SO}_2$ , or the like; in order to prevent the introduction of active oxygen from the air into the fixing chamber.

The invention is further described by reference to the accompanying drawings of which Fig. 1 is a cross-section and Fig. 2 a longitudinal section through a furnace adapted or altered to carry on the process. Like reference numerals refer to like parts in both figures. In Fig. 1 the ore to be treated is fed so as to form a sloping embankment resting upon the floor and against the walls of the furnace chamber. This ore is sulphide material and is oxidized by forcing air through the tuyères 1 upon the sides of the furnace chamber and saturating the embankment with oxygen. When air is used it impinges from the tuyère into the heated sulphide material and oxidizes the sulphur to  $\text{SO}_2$ . This  $\text{SO}_2$  passes from the embankment into the furnace chamber and as it does so it progresses into a temperature where it breaks into elemental sulphur and oxygen and is mixed with the furnace gas. The oxygen set free from  $\text{SO}_2$  by high temperature is fixed by spraying into it oxidizable materials such as sulphide ores, coal dust, powdered peat, sawdust and like material or sulphide ores through pipes shown at 2, Fig. 2. When oil vapor or powdered coal or the like is used to fix the oxygen it is sprayed in through 2, near the point of the flame 4, where combustion of the fuel at the firing end of the furnace is complete and the balance of the furnace chamber is kept filled with oxidizable fume

or vapor which passes out the flue 5 to the precipitating or dust chamber.

Having thus described my invention, what I claim as new and desire to secure by

5 Letters Patent is:

1. A method of treating materials yielding sulphur-dioxide upon oxidation and preventing the production of the sulphur-dioxide consisting of treating said materials 10 within a temperature where sulphur-dioxide dissociates into sulphur and oxygen and fixing said oxygen while dissociated from said sulphur with an oxidizable material.
2. A method of treating sulphide ores con-

sisting of preparing said ores in a fine state 15 of division and spraying them into dissociated sulphur and oxygen and oxidizing the metal content of said ores with the oxygen dissociated from said sulphur.

3. A method of oxidizing metal sulphides 20 which consists of introducing them in a divided condition into a gas mixture produced by heating an oxide of sulphur to dissociation.

GEORGE CAMPBELL CARSON.

Witnesses:

S. E. BRETHERTON,  
FLORA HALL.